# EUROPEAN PATENT APPLICATION

(11) **EP 2 314 401 A1**
(43) Date of publication of application: **27.04.2011**
(21) Application number: 10172843.4
(22) Date of filing: 13.08.2010
(51) Int. Cl.: B22F 3/03, B29C 33/00

(54) **Mould design and powder moulding process**

(30) Priority: 09.09.2009 US 240828 P
(71) Applicant: DePuy Products, Inc., Warsaw, IN 46581 (US)
(72) Inventor: Liu, Hengda Derek, Warsaw, IN 46580 (US); Martin, Andrew James, Warsaw, IN 46236 (US); Rim, Juwan, 120-190 Seoul (KR); Rybolt, Jeffrey A, Fort Wayne, IN 46804 (US)
(74) Representative: Belcher, Simon James

(57) **Abstract**

A mould comprises a substantially concave portion, and a cap portion that is configured for removable attachment to the substantially concave portion and comprises a mandrel formed from a substantially rigid material. The cap portion and the substantially concave portion, when attached, define an internal space having a three-dimensional shape.

## Description

The present invention relates to, among other things, methods and devices for the preparation of porous metal constructs.

Cold isostatic pressing is an effective way to prepare near net shaped powder compacts. The process involves filling moulds with powders, and placing the filled moulds in a pressure vessel that is used to compress the powder into a compacted mass (green body). A cold isostatic press is often used to compress powder mixtures of metal and space filler, wherein the latter is removed following compaction to obtain a metal structure having pores. Porous metal constructs are widely used as, among other things, orthopaedic implants, supports for catalysts, bone growth substrates, and filters.

Traditional methods of preparing powder compacts have involved the filling of an assembled mould, the interior space of which substantially corresponds to the shape of the green body that results from compacting the powder with which the mould is filled. The assembled moulds are filled by pouring the metallic powder or powder mixture through a small opening in the mould that is subsequently plugged prior to compaction. For example, a mould that is designed for preparing a metal construct in the form of an acetabular cup typically features an end cap and a dome, wherein the peak of the dome includes a hole into which a powder may be poured in order to fill the mould. After filling, a plug is used to seal the mould before compaction commences.

However, conventional moulds of this variety can produce unsatisfactory results in a number of respects. For example, there is often dimensional variability among the green bodies that are produced by subjecting the filled moulds to pressure; in the case of cup-shaped moulds, for example, the inner and outer radii of the cup can respectively vary from green body to green body.

Another problem is that filling the mould through a small hole and using a plug to seal the mould can result in an imperfection in the resulting green body at the location of the plugged opening.

The process of filling such moulds is also difficult and time-consuming to perform. Typically, after the mould is filled through the opening with as much powder as possible, the mould is closed and tapped against a hard surface in order to cause the powder to settle as much as possible. The fill hole so that more powder can be introduced; this process is repeated until the mould is as completely filled as possible. Aside from being bothersome and protracted, the filling process can result in powder spillage, which causes waste and risks the possibility of exposure of personnel to escaped powder. In addition, despite such efforts, the process often results in an imperfectly filled mould.

Overfilling of the mould with powder can cause the formation of gaps between parts of the mould. Compaction of a filled mould may involve the use of water as a compression medium, leading to leakage of water, especially when the mould has been overfilled. Such leakage can lead to failure in attempts to form a compacted body.

A further problem with conventional moulds is that repeated usage often causes wear on the mandrel section of the end cap relative to the other portions of the mould. If the shape of the mandrel is altered as a result of wear, the green body that is produced in the worn mould can deviate from the desired shape. Excessive wearing of the mandrel can also lead to cracking and splitting on that part of the mould.

There exists a need for moulds that are designed to overcome some or all of such problems and that are capable of endowing the compaction process with uniformity and repeatability.

In one aspect, the present invention provides moulds that comprise a substantially concave portion, and a cap portion that is configured for removable attachment to the substantially concave portion, wherein the cap portion and the substantially concave portion, when attached, define an internal space having a three-dimensional shape, and wherein the cap portion comprises a mandrel that is formed from a substantially rigid material and is disposed on a surface of the cap portion defining the internal space.

In another aspect, the present invention provides a moulding method comprising providing a mould that comprises a substantially concave portion and a cap portion that is configured for removable attachment to the substantially concave portion, placing metal powder into the substantially concave portion, and attaching the cap portion to the substantially concave portion following the placement of the metal powder therein.

The invention also provides a moulding method which comprises placing a metal powder into a substantially concave portion of a mould, wherein the mould further comprises a cap portion that is configured for removable attachment to the substantially concave portion and comprises a mandrel formed from a substantially rigid material, and compacting the mould to form a green body comprising the metal powder.

Optionally, the metal powder is placed into the substantially concave portion of the mould prior to attachment of the cap portion to the substantially concave portion, and further comprising attaching the cap portion to the substantially concave portion prior to compacting the mould.

Optionally, the metal powder is placed into the substantially concave portion of the mould while the cap portion is attached to substantially concave portion.

Optionally, the metal powder is placed into the substantially concave portion of the mould through an opening in the substantially concave portion.

Optionally, the cap portion and the substantially concave portion, when attached, define an internal space having a three-dimensional shape.

Optionally, the cap portion and the substantially concave portion, when attached, define an internal space having a substantially hollow hemispherical shape.

The present invention provides, among other things, devices and methods for the preparation of structures comprising compacted particles, such as green bodies that are prepared from powders, including metallic powders. The disclosed methods and devices typically provide more uniform and repeatable compaction than conventional moulds, and can be used to produce, for example, compacted structures having more dimensionally accurate and repeatable surface features, thereby yielding a better, more optimal near net shaped part. In addition, the invention provides methods and devices that in certain embodiments are compatible with rapid and consistent filling of moulds with powders. These advantages and others will become more readily apparent from the detailed description provided below.

The invention provides moulds that comprise a substantially concave portion, and a cap portion that is configured for removable attachment to the substantially concave portion, wherein the cap portion and the substantially concave portion, when attached, define an internal space having a three-dimensional shape, and wherein the cap portion comprises a mandrel that is formed from a substantially rigid material and is disposed on a surface of the cap portion defining the internal space.

A cold isostatic press is often used to compact powders or powder mixtures, including metal powders, in conventional moulds. FIG. 1 is a view of a conventional mould 2 which is disassembled. Such moulds are typically made from rubber and can comprise an end cap 4 having a mandrel 6, and a main body 8 that includes an opening 10 into which the powder or powder mixture is poured in order to fill the mould when the main body 8 and end cap 4 are assembled into the mould 2. To assemble the mould, the main body 8 is secured over end cap 4, with the mandrel 6 positioned within the internal space of mould 2. Ribs 14 on the outer edge of end cap 4 form a seal with the inner face of the end 16 of main body 8. After the assembled mould is filled, opening 10 is sealed using a plug 12 prior to compaction of the filled mould 2.

There is often some dimensional variability among compacted parts that are made with conventional moulds, due in part to the flexibility of the material of which the mould is made. However, it has been discovered that incorporating a mandrel that is formed from a substantially rigid material into the end cap of a mould significantly improves the repeatability of the compression process, allowing for the preparation of precisely and accurately shaped compressed parts with each use of the mould. This repeatability also provides a basis for accurate machining of the compressed part (green body); in the absence of such repeatability, it is difficult to position the green body for accurate machining and thereby to produce precisely formed end parts. In addition, to the extent that the green bodies that are produced using mandrel cap moulds as provided by the invention approximate the shape of the internal space defined by the parts of the assembled mould more reliably, less machining is necessary, which conserves time and energy, and also reduces powder wastage.

The inclusion of a mandrel that is formed from a substantially rigid material also assists the mould in resisting wear. Conventional moulds deteriorate after repeated use, and the present inventors have discovered that splitting and cracking of flexible mandrels occurs long before any perceptible wear appears on the mandrels of moulds as provided by the invention. Therefore, the use of a mandrel that is formed from a substantially rigid material can improve mould life which is important because a worn mould can admit water during a cold isostatic press procedure. Leakage of water into the mould can damage or destroy the part, and can cause powder to enter the pressure chamber. Accordingly, moulds provided by the invention can in many instances increase mould life, decrease the incidence of wasted parts, and improve the safety of the process of preparing green bodies from powder materials.

It has also been discovered that the present moulds can often produce green bodies from powder mixtures with reduced segregation among different particle types. Such results are described in Example 2, below. Evenness of particle dispersion provides for more uniform porosity in the finished construct, as well as enhanced uniformity with respect to other structural attributes.

The internal space of the assembled moulds may define any three dimensional shape, and preferably defines a three dimensional shape that substantially corresponds to the shape of a medical implant, catalyst, or other structure that is to be prepared from the green body. For example, the three dimensional shape of the internal space that is defined by the assembled mould may have a substantially hollow, hemispherical shape. moulds having an internal space that have a substantially hollow, hemispherical shape may be used to form green bodies that can, in turn, be made into acetabular cup orthopaedic implants.

The moulds may be filled in accordance with conventional techniques, i.e., by pouring a fill material, such as a metal powder or mixture of powders, into an opening in the assembled mould. For example, the substantially concave portion may comprise an opening that is configured for receiving a metal powder for filling the mould. Once the mould has been filled, the opening may be plugged prior to compaction. In other embodiments, the substantially concave portion does not include an opening, and the mould is not filled in the assembled state. Such embodiments are more fully described in this specification.

The cap portion comprises a mandrel that is formed from a substantially rigid material. The substantially rigid material may be any substance or mixture of substances that render the mandrel more rigid than a conventional flexible mandrel (for example, a rubber mandrel). Preferably, the mandrel may comprise any material that can withstand pressures of about 137.9 to about 413.7 MPa (about 20 to about 60 ksi) with limited deformation. As used herein "limited deformation" preferably refers to deformation that is less than about 0.5%, less then about 0.3%, less than about 0.2%, or less than about 0.1%. The substantially rigid material may be, for example, a metal, a metal alloy, a ceramic or a synthetic polymer. Examples of suitable polymers include polypropylene, polyetherether-ketone, polyphenylsulfone, polyetherimide and their carbon-fibre reinforced or glass-fibre reinforced counterparts. Examples of suitable metals include stainless steel, carbon steel, alloy steel, titanium, a titanium alloy (e.g., Ti-6Al-4V), a cobalt-chromium alloy, aluminum or an aluminum alloy, molybdenum, tantalum, niobium, zirconium, tungsten, or any combination thereof. Examples of suitable ceramics include alumina, zirconia, carbides, nitrides, borides, and silicides. The mandrel may be any three dimensional geometric or irregular shape. For example, the mandrel may be substantially hemispherical, substantially cube shaped, substantially cone shaped, substantially pyramidal, substantially cylindrical, or shaped like another regular or irregular three dimensional geometric object.

The end cap may include one or more aspects that are substantially concave. However, in many embodiments the substantially concave portion of the mandrel cap moulds provided by the invention is configured such that it would hold a greater volume of fill material than the end cap if the volumetric capacities of the respective parts were compared. The substantially concave portion may be hemispherical. For example, the substantially concave portion may literally be a hemisphere (a half-sphere), or may be a lesser or greater portion of a sphere or other spheroidal body such as an ovoid. The substantially concave portion may be a three dimensional object, such as a polyhedron. Thus, the substantially concave portion may be substantially cube shaped, substantially rectangular prismatic, substantially cylindrical, substantially cone shaped, substantially pyramidal, or shaped like another regular or irregular three dimensional geometric object.

The substantially concave portion may be formed from flexible material. In these and other embodiments, the cap portion may comprise flexible material that is fixedly attached to the mandrel. When the cap portion comprises flexible material that is fixedly attached to the mandrel, the flexible material may comprise a ring that is fixedly attached to an outer edge of the mandrel. Because the outer edge of the mandrel may be any shape (depending on the shape of the mandrel itself), a "ring" may refer to any shape having an inner edge that substantially conforms to the shape of the outer edge of the mandrel, and having an outer edge that substantially conforms to the shape of the inner or outer edge of the substantially concave portion. As used herein, a "flexible" material is one that is pliable relative to a substantially rigid material such as steel. Conventional mould components are often rubber, and the substantially concave portion, the part of the cap portion that is fixedly attached to the mandrel, or both, may be conventional rubber (natural or synthetic) or another material having similar properties. Other possible materials include, inter alia, polyisoprene, neoprene, chloroprene, silicone, polyvinyl chloride (PVC), nitrile, vinyl acetate, ethylene propylene diene M-class rubber (EPDM), fluorinated hydrocarbon or a fluoroelastomer (such as that sold under the trade mark Viton by DuPont Performance Elastomers, Wilmington, DE), crosslinked polyethylene (XLPE), butyl rubber, fluorosilicone rubber, polyurethane, and the like. The physical dimensions of the flexible material of the substantially concave portion and of the cap portion may each vary as dictated by the particular requirements of the user. For example, the flexible material of the substantially concave portion and of the cap portion independently can be between about 0.76 and about 12.7 mm (about 0.03 and about 0.50 inch) thick. In other embodiments, the thickness of the flexible material of either component can be between about 0.76 and about 7.62 mm (about 0.05 and about 0.30 inch), between about 2.54 and about 5.1 mm (about 0.10 and about 0.20 inch), or about 3.2 mm (about 0.125 inch).

The cap portion of the mould is configured for removable attachment to the substantially concave portion and comprises a mandrel formed from a substantially rigid material. The configuration of the cap portion so that it can be removably attached to the substantially concave portion may be in accordance with conventional designs, with which those of ordinary skill in the art are familiar. FIG. 1 depicts a conventional end cap 4, which includes ribs 14 that form a seal with the inner face of the end 16 of main body 8 when mould 2 is in its assembled state. In other embodiments, the perimeter of the cap portion may comprise a lip that seals against the outer edge of the substantially concave portion. FIG. 2A shows an end cap 18 which can be used in a mandrel cap mould as provided by the present invention. The nd cap 18 comprises a mandrel 20 that comprises a substantially rigid material, and a ring 22 of flexible material that is fixedly attached to the outer edge of the mandrel 20. FIG. 2B is a cross sectional view of the end cap 18 shown in FIG. 2A, in which the end cap 18 is removably attached to a substantially concave portion 26. At its outermost edge, ring 22 of flexible material terminates in a lip 24 that is configured for removable attachment to the outer edge of one end of the substantially concave portion 26. In this manner, the end cap 18 is interlocked with the substantially concave portion 26 in such a manner as to form a secure seal between the components of the mould. The removable fixation of end cap 18 by means of the lip 24, or by other means in accordance with other embodiments, provides a seal that, among other things, prevents water from entering the mould during the compaction process and prevents powder from escaping from the internal space of the mould into the compression chamber. The removable fixation of the end cap to the substantially concave portion may be achieved in any appropriate manner, such as by providing any suitable overlap or interlock between them.

The invention provides methods comprising providing a mould that comprises a substantially concave portion and a cap portion that is configured for removable attachment to the substantially concave portion, placing metal powder into the substantially concave portion; and attaching the cap portion to the substantially concave portion following the placement of the metal powder therein. Such methods employ a particular embodiment of mandrel cap mould, as described above, in which the substantially concave portion does not include an opening, and the mould is not filled in the assembled state. Rather, the mould is filled by placing metal powder into the substantially concave portion prior to attachment to the end portion. In accordance with such methods, a desired quantity of metal powder (in particular, an amount that is known to precisely fill the mould) is determined by weight, i.e., by weighing out the powder on a suitable instrument, such as a laboratory scale. When the desired quantity of powder has been obtained, the powder is placed into the substantially concave portion. FIG. 3A shows an example of substantially concave portion 28 that is filled with powder 30 while separated from an end cap 32. As shown in FIG. 3B, when the powder 30 has been placed into the substantially concave portion 28, end cap 32 is joined to the substantially concave portion 28, whereupon powder 30 is housed within the mould. The use of a precise amount of powder that is suitable for use in the generally concave portion precludes a situation whereby too much powder (i.e., overfilling of the mould, which can make it difficult to assemble the mould properly and/or can cause the parts of the mould to separate during compression) or too little powder (i.e., underfilling of the mould, which can prevent the resulting green body from having the proper shape) is placed in the substantially concave powder. The method provided by the invention may include the step of compacting the mould to form a green body comprising the metal powder. The ability to place a desired quantity of powder into the substantially concave portion prior to assembly of the mould ensures a higher degree of consistency among the green bodies that are formed by compacting the assembled mould, enables the creation of a more near net shaped part, and improves the process of machining.

The invention provides methods comprising placing a metal powder into a substantially concave portion of a mould, wherein the mould further comprises a cap portion that is configured for removable attachment to the substantially concave portion and comprises a mandrel formed from a substantially rigid material, and compacting said mould to form a green body comprising the metal powder. In accordance with such methods, the metal powder may be placed into the substantially concave portion of the mould prior to attachment of the cap portion to the substantially concave portion. In such embodiments, the method may further comprise attaching the cap portion to the substantially concave portion prior to compacting the mould. In other embodiments, the metal powder is placed into the substantially concave portion of the mould while the cap portion is attached to substantially concave portion. For example, the metal powder may placed into the substantially concave portion of the mould through an opening in the substantially concave portion. After the metal powder is placed into the mould, the opening in the substantially concave portion may be closed, e.g., using a plug, and remains closed during compaction of the filled mould in order to form a green body.

With respect to any of the methods disclosed herein, the metal powder may comprise one or more metals, optionally in combination with an extractable material. The extractable material may be included in order to form a porous construct pursuant to the "space holder" method. The space holder method is a well known process for making metallic foam structures and employs dissolvable or otherwise removable space-holding materials that are combined with metallic powders and subsequently removed from the combination by various methods, including heat or liquid dissolution, leaving behind a porous matrix formed from the metallic powder. The porous matrix material is then sintered to further strengthen the matrix structure. Numerous variations on the space holder concept are known, for example as disclosed in US-3852045, US-6849230, US-A-2005/ 0249625 and US-A-2006/0002810.

The metal powder, and by extension the resulting green body and porous construct, may comprise any biocompatible metal, examples of which include titanium, a titanium alloy (e.g., Ti-6Al-4V), a cobalt-chromium alloy, aluminum, molybdenum, tantalum, magnesium, niobium, zirconium, stainless steel, nickel, tungsten, or any combination thereof. In accordance with known methods for forming green bodies and porous constructs using metal powders, it will be readily appreciated that the metal powder particles may be substantially uniform or may constitute a variety of shapes and sizes, e.g., may vary in terms of their three-dimensional configuration and/or may vary in terms of their respective major dimension. Measured with respect to a given particle's major dimension, particle size may be from about 20 µm to about 100 µm, from about 25 µm to about 50 µm, or from about 50 µm to about 80 µm. The metal powder particles may be spheroids, roughly cylindrical, platonic solids, polyhedrons, plate- or tile-shaped, irregularly shaped, or any combination thereof. In preferred embodiments, the metal powder comprises particles that are substantially similarly shaped and substantially similarly sized.

The extractable material may be a material that is soluble in an aqueous fluid, an organic solvent, a combination of such solvents, or any other suitable solvent. The material may comprise a salt, a sugar, a solid hydrocarbon, a urea derivative, a polymer, or any combination thereof. Examples include ammonium bicarbonate, urea, biuret, melamine, ammonium carbonate, naphthalene, sodium bicarbonate, sodium chloride, ammonium chloride, calcium chloride, magnesium chloride, aluminum chloride, potassium chloride, nickel chloride, zinc chloride, ammonium bicarbonate, sodium hydrogen phosphate, sodium dihydrogen phosphate, potassium dihydrogen phosphate, potassium hydrogen phosphate, potassium hydrogen phosphite, potassium phosphate, magnesium sulphate, potassium sulphate, alkaline earth metal halides, crystalline carbohydrates (including sucrose and lactose or other materials classified as monosaccharides, disaccharides, or trisaccharides), polyvinyl alcohol, polyethylene oxide, a polypropylene wax (such those available from Micro Powders, Inc., Tarrytown, NY under the PROPYLTEX trade mark), sodium carboxymethyl cellulose (SCMC), or any combination thereof. Alternatively or additionally, the extractable material may be removed under heat and/or pressure conditions; for example, the extractable material may volatilize, melt, or otherwise dissipate as a result of heating. Examples of such extractable materials include ammonium bicarbonate, urea, biuret, melamine, ammonium carbonate, naphthalene, sodium bicarbonate, and any combination thereof.

When the extractable material comprises particles, such particles may be substantially uniform with respect to one another or may constitute a variety of shapes and sizes, e.g., may vary in terms of their three-dimensional configuration and/or may vary in terms of their respective major dimension. The extractable material can be present in a wide variety of particle sizes and particle size distributions suitable to produce a desired pore size and pore size distribution. Certain preferred particle size ranges are from about 200 µm to about 600 µm, from about 200 µm to about 300 µm, and from about 425 µm to about 600 µm. The extractable material particles may be spheroids, roughly cylindrical, platonic solids, polyhedrons, plate- or tile-shaped, irregularly shaped, or any combination thereof. In preferred embodiments, the space filler comprises particles that are substantially similarly shaped and substantially similarly sized. Because the size and shape of the pores of the porous construct that is eventually produced from the mixture of the metal powder and the extractable material roughly correspond to the size and shape of the particles of the extractable material, one skilled in the art will readily appreciate that the characteristics of the particles of the extractable material may be selected according to the desired configuration of the pores of the resulting porous product. In accordance with the present invention, when the extractable material comprises particles that are substantially similarly shaped and substantially similarly sized, the porosity of a porous construct that is eventually formed using the extractable material of this type will be substantially uniform.

A powder mixture may comprise metal powder in an amount that is about 5% by volume to about 45% by volume, preferably about 15% by volume to about 40% by volume, the balance of the powder mixture comprising the extractable material. Once the extractable material is removed from the green body that is formed from the mixture of the metal powder and extractable material in later stages of the present methods, the resulting porosity of the green body may be about 55% to about 95%, preferably about 60% to about 85%. The powder mixture of which the green body is made may comprise about 18 wt.% to about 67 wt.% metal powder, the balance of the powder mixture comprising the extractable material.

Suitable techniques for mixing a metal powder with an extractable material are known, for example as disclosed in US-3852045, US-6849230, US-A-2005/0249625 and US-A-2006/0002810. Ideally, the mixing results in a substantially uniform dispersion of the particles comprising the minor component of the powder mixture among the particles comprising the major part of the powder mixture. The metal powder may comprise about 18 to about 67 wt.% of the powder mixture, the balance of the powder mixture comprising the extractable material. Once the extractable material is removed from the green body in later stages of the present methods, the resulting porosity of the green body may be about 50% to about 90%, preferably about 60% to about 85%. The removal of the extractable material is described more fully in WO-A-2009/143420.

The mould need not be designed to produce near-net shape parts or parts whose moulded form resembles the desired final, sintered part; moulds may produce generic shapes, such as bars, rods, plates, or blocks, that may be subsequently machined in the green state to produce a part that after sintering-induced shrinkage closely approximates the desired shape of the final product, with optional machining of the sintered part. moulds and mould assemblies for such purposes are well known among those skilled the art and may allow for the preparation of bodies that are, for example, spherical, spheroid, ovoid, hemispherical, cuboid, cylindrical, toriod, conical, concave hemispherical (that is, generally cup-shaped), irregular, or that adopt any other desired three-dimensional conformation. Once formed from the powder or powder mixture in accordance with the preceding, the resulting shaped object may be compacted to form the green body. The shaped object is compacted while contained within a mould assembly. Compacting may be uniaxial, multi-axial, or isostatic. In preferred embodiments, a cold isostatic press is used to compact the powder into the green body. Following the compacting procedure, the resulting green body may be removed from the mould and may be processed. Processing may include machining or otherwise refining the shape of the green body.

### Example 1 - Acetabular Cup

Green bodies for forming acetabular cup orthopaedic devices were made from a conventional mould and from a mandrel cap mould as provided by the present invention. The conventional mould included an end cap 4 and substantially concave portion 8 as depicted in FIG. 1. The mandrel cap mould included an end cap 18 as shown in FIG. 2A, including a mandrel 20 that comprises a substantially rigid material, and a ring 22 of flexible material that is fixedly attached to the outer edge of the mandrel 20. The mould also included a substantially concave portion 28 as shown in FIG. 3A.

The conventional mould was filled affixing end cap 4 to substantially concave portion 8, and by pouring a metal powder comprising titanium or titanium alloy mixed with extractable material into the opening 10 of the substantially concave portion 8. Because the opening 10 was confined and small, a funnel was used to pour the powder into the mould. Even with the use of a funnel, some air remained within the mould during the filling process. In order to fill up the mould as completely as possible with the mixed powder, multiple steps were performed during which time the mould was shaken or vibrated repeatedly during pauses between bouts of scoop feeding the powder into the mould. The opening 10 was then sealed using a stopper 12, and the mould was placed into the compression chamber of the pressure vessel (Cold Isostatic Press, CIP42260, Avure Autoclave Systems, Inc., Kent, WA), which was filled with water as the pressure medium. The pressure vessel was closed in accordance with standard procedure, and the contents of the vessel, including the mould, were subjected to cold isostatic pressing at a pressure of 310 MPa (45 ksi) for about 15 seconds. The pressure vessel was then opened and the mould was removed. The mould was then disassembled and the compacted metal part was extracted.

The mandrel cap mould was filled by weighing out, for example, 131.9 g of a metal powder comprising titanium mixed with sodium chloride on an electronic scale (XS16001L Precision Balance, Mettler-Toledo, Inc., Columbus, OH), and pouring the weighed aliquot of metal powder into substantially concave portion 28. The mould was closed by affixing end cap 18 to the substantially concave portion 28. The mould was placed into the compression chamber of the pressure vessel (Cold Isostatic Press, CIP42260, Avure Autoclave Systems, Inc., Kent, WA) which was filled with water as the pressure medium. The pressure vessel was closed in accordance with standard procedure, and the contents of the vessel, including the mould, were subjected to cold isostatic pressing at a pressure of 310 MPa (45 ksi) for about 15 seconds. The pressure vessel was then opened and the mould was removed. The mould was then disassembled and the compacted metal part was extracted.

FIG. 4A depicts a photographic image of the green body 34 that was removed from the conventional mould, while FIG. 4B provides a photographic image of the green body 38 that was removed from the mandrel cap mould. A visual analysis of the compacted parts reveals that green body 34 was not a true hemisphere, and the dispersion of particles therein was non-uniform. Because a conventional mould possessed a small, confined opening, it was necessary to fill the mould scoop by scoop in small amounts, which became progressively more difficult as the mould became closer to being filled to capacity: the mould must be shaken, vibrated or pounded on a counter during filling, which resulted in the drying and segregation of the powder mixture as between the metal particles and space holder material. In FIG. 4A, the darker bands on green body 34 are indicative of portions that contain a higher proportion of metal powder relative to space holder material, and lighter bands indicate portions that have a higher proportion of space filler material relative to metal powder. In addition, green body 34 included a blemish 36 that corresponds to the location of the opening in the substantially concave portion that receives the metal powder during the filling of the mould. In contrast, green body 38 more closely approximated a true hemisphere, featured uniform particle dispersion, and had a substantially smooth surface profile. Cup dimension measurements of the green state parts that result from the use of the two moulds are set out in Table 1 (with "R" and "H" measured as shown in FIG. 5).

**TABLE 1**

| Measurement | Conventional mould | | | Mandrel cap mould | | |
|---|---|---|---|---|---|---|
| | R (mm) | H (mm) | R-H (mm) | R (mm) | H (mm) | R-H (mm) |
| 1 | 32.35 | 27.85 | 4.50 | 28.03 | 28.89 | -0.86 |
| 2 | 32.61 | 27.84 | 4.77 | 28.02 | 28.94 | -0.92 |
| 3 | 32.42 | 27.75 | 4.67 | 28.09 | 28.93 | -0.84 |
| 4 | 32.65 | 27.86 | 4.79 | 28.11 | 28.89 | -0.78 |
| 5 | 32.33 | 27.70 | 4.63 | 28.04 | 28.92 | -0.88 |
| 6 | 32.49 | 27.83 | 4.66 | 28.13 | 28.89 | -0.76 |
| 7 | 32.04 | 27.88 | 4.16 | 28.05 | 28.93 | -0.88 |
| 8 | 32.17 | 27.79 | 4.38 | 28.03 | 28.92 | -0.89 |
| Mean | 32.38 | 27.81 | 4.57 | 28.06 | 28.91 | -0.85 |
| Std dev | 0.21 | 0.06 | 0.21 | 0.04 | 0.02 | 0.06 |

Standard deviation values were greater for the green bodies prepared using conventional moulds than those prepared using mandrel cap moulds. In addition, with respect to the cups that were prepared using mandrel cap moulds as provided by the invention, the variation between the "R" and "H" radius values (expressed as "R-H") was considerably less than that which was measured with respect to the cups that were prepared using conventional moulds. This indicates that the use of the present moulds allows for the preparation of green bodies that come much closer to resembling a true approximation of the mould shape than do the green bodies made using conventional moulds.

### Example 2 - Repeatability

The mandrel cap moulds were tested for the ability to consistently produce green bodies having a predictable shape and particle dispersion. A single mould for an acetabular cup was filled and subjected to compaction in accordance with the conditions described in Example 1, above, and this process was repeated three times in order to obtain three separate green bodies. The green bodies were compared by visual inspection and physical measurement. It was found that the green bodies that were produced using the mould were of substantially uniform shape and did not include blemishes or other physical discrepancies that would be expected among green bodies that are produced using conventional moulds. Table 2, below, provides data demonstrating that the standard deviations among the R, H, and R-H values that are measured with respect to green bodies that are produced using mandrel cap moulds (0.020, 0.23, and 0.26, respectively) are less than those which are measured with respect to green bodies that are produced using conventional moulds (0.31, 0.94, and 0.90, respectively).

**TABLE 2**

| Sample number | Measurement | Conventional mould | | | Mandrel cap mould | | |
|---|---|---|---|---|---|---|---|
| | | R (mm) | H (mm) | R-H (mm) | R (mm) | H (mm) | R-H (mm) |
| 1 | 1 | 32.02 | 26.86 | 5.16 | 37.20 | 36.82 | 0.38 |
| | 2 | 32.45 | 26.73 | 5.72 | 37.03 | 36.42 | 0.61 |
| | 3 | 31.48 | 27.05 | 4.43 | 37.39 | 37.13 | 0.26 |
| | 4 | 32.05 | 27.47 | 4.58 | 37.35 | 36.83 | 0.52 |
| 2 | 1 | 32.11 | 29.07 | 3.04 | 37.65 | 36.97 | 0.68 |
| | 2 | 32.56 | 29.06 | 3.50 | 37.51 | 36.45 | 1.06 |
| | 3 | 32.02 | 29.40 | 2.62 | 37.50 | 36.42 | 1.08 |
| | 4 | 32.17 | 29.06 | 3.11 | 37.55 | 36.74 | 0.81 |
| 3 | 1 | 31.95 | 28.32 | 3.63 | 37.16 | 36.72 | 0.44 |
| | 2 | 32.53 | 28.50 | 4.03 | 37.53 | 36.83 | 0.70 |
| | 3 | 31.93 | 28.37 | 3.56 | 37.61 | 36.74 | 0.87 |
| | 4 | 32.39 | 28.52 | 3.87 | 37.54 | 36.96 | 0.58 |
| | Mean | 32.14 | 28.20 | 3.94 | 37.42 | 36.75 | 0.67 |
| | Std dev | 0.31 | 0.94 | 0.90 | 0.20 | 0.23 | 0.26 |

FIG. 6A shows images of green bodies 40, 42, 44 that were produced using mandrel cap moulds as provided by the invention. Like the green body shown in FIG. 4B, green bodies 40, 42, 44 approximated a true hemisphere, featured uniform particle dispersion, and had a substantially smooth surface profile. FIG. 6A also demonstrates that the moulds of the present invention produce green bodies that are of substantially uniform shape from green body to green body, and that do not include blemishes or other physical discrepancies that would be expected among green bodies that are produced using conventional moulds. In comparison, FIG. 6B shows that green bodies 46, 48, 50, 52 that were produced using conventional moulds varied from one another with respect to the parameters of shape, surface profile, and particle dispersion.

In this document, the singular forms "a," "an," and "the" include the plural reference, and reference to a particular numerical value includes at least that particular value, unless the context clearly indicates otherwise. Thus, for example, a reference to "a powder" is a reference to one or more of such powders and equivalents thereof known to the skilled reader. When values are expressed as approximations, by use of the antecedent "about," it will be understood that the particular value forms another embodiment. As used herein, "about X" (where X is a numerical value) preferably refers to ±10% of the recited value, inclusive. For example, the phrase "about 8" preferably refers to a value of 7.2 to 8.8, inclusive; as another example, the phrase "about 8%" preferably refers to a value of 7.2% to 8.8%, inclusive (rounded to the nearest integer in cases where integral quantities are considered). Where present, all ranges are inclusive and combinable. For example, when a range of "1 to 5" is recited, the recited range should be construed as including ranges "1 to 4", "1 to 3", "1-2", "1-2 & 4-5", "1-3 & 5", "2-5" , and the like. In addition, when a list of alternatives is positively provided, such listing can be interpreted to mean that any of the alternatives may be excluded, e.g., by a negative limitation in the claims. For example, when a range of "1 to 5" is recited, the recited range may be construed as including situations whereby any of 1, 2, 3, 4, or 5 are negatively excluded; thus, a recitation of "1 to 5" may be construed as "1 and 3-5, but not 2", or simply "wherein 2 is not included."

Unless otherwise specified, the characteristics of the components or steps that are described with respect to one embodiment of the invention are applicable to the components or steps of other embodiments of the invention.

## Claims

1. A mould comprising:
a substantially concave portion; and,
a cap portion that is configured for removable attachment to the substantially concave portion,
in which the cap portion and the substantially concave portion, when attached, define an internal space having a three-dimensional shape, and in which the cap portion comprises a mandrel that is formed from a substantially rigid material and is disposed on a surface of the cap portion defining the internal space.

2. The mould according to claim 1 in which the substantially concave portion comprises an opening that is configured for receiving a metal powder.

3. The mould according to claim 1 in which the substantially concave portion is hemispherical.

4. The mould according to claim 3 in which the cap portion and the substantially concave portion, when attached, define an internal space having a substantially hollow hemispherical shape.

5. The mould according to claim 1 in which the substantially concave portion is formed from a flexible material.

6. The mould according to claim 1 in which the substantially rigid material comprises metal.

7. The mould according to claim 1 in which the cap portion comprises flexible material that is fixedly attached to the mandrel, in which the

8. The mould according to claim 7 in which the flexible material of the cap portion comprises a ring that is fixedly attached to an outer circumference of the mandrel.

9. A moulding method comprising:
providing a mould that comprises a substantially concave portion and a cap portion that is configured for removable attachment to the substantially concave portion,
placing metal powder into the substantially concave portion; and
attaching the cap portion to the substantially concave portion following the placement of the metal powder therein.

10. The method according to claim 9 in which the cap portion and the substantially concave portion, when attached, define an internal space having a three-dimensional shape.

11. The method according to claim 10 in which the cap portion and the substantially concave portion, when attached, define an internal space having a substantially hollow hemispherical shape.

12. The method according to claim 10 in which the cap portion comprises a mandrel formed from a substantially rigid material.

13. The method according to claim 9 further comprising compacting the mould to form a green body comprising the metal powder.
